

# UNITED STATES PATENT OFFICE.

HENRY HAYNES, OF PHILADELPHIA, PENNSYLVANIA.

## INSULATING COMPOUND FOR PRINTING-PRESSES.

SPECIFICATION forming part of Letters Patent No. 508,107, dated November 7, 1893.

Application filed April 29, 1893. Serial No. 472,413. (No specimens.)

*To all whom it may concern:*

Be it known that I, HENRY HAYNES, a subject of the Queen of Great Britain, residing in the city and county of Philadelphia, State 5 of Pennsylvania, have invented a new and useful Improvement in Insulating Compounds for Printing-PresSES, which improvement is fully set forth in the following specification.

My invention consists of a compound where-  
10 by the tympan sheet or other proper part of a printing press may be insulated, and the paper to be printed is prevented from being electrically charged, thus producing superior results, as will be hereinafter set forth.

15 In carrying out my invention, I take machine, petroleum or equivalent oil one gallon; glycerine, one quart; paraffine wax, three quarters of an ounce; castor oil, two ounces. The proportions may however be varied ac-  
20 cording to requirements. The oils and wax are heated until the wax is thoroughly dissolved, and the mass is stirred, and when cold the glycerine is added, and all well mixed together.

25 To use the compound it is well shaken and applied to the tympan sheet of the press, it being spread evenly over said sheet, a little larger than the form. Some waste sheets are

now passed through the press so as to remove the superfluous compound which has not been 30 absorbed by the tympan sheet.

In cold weather there is more or less electricity in the paper to be printed, which causes trouble, such as the paper sticking to the fly, or being thrown on the floor, offsetting on the 35 back of the paper, and difficulty of separation. By using my composition the trouble will be overcome, as the tympan sheet and paper will be insulated, and the paper will be delivered straight and even, and what has 40 been printed on one side may be printed on the other side. As the paper runs so well through the press, the latter may be operated at a higher rate of speed, and thus produce 45 more work.

Having thus described my invention, what I claim as new, and desire to secure by Letters Patent, is—

An insulating compound for a printing press composed of machine oil, wax, glycerine, 50 and castor oil, substantially as described.

HENRY HAYNES.

Witnesses:

JOHN A. WIEDERSHEIM,  
WM. C. WIEDERSHEIM.